# EUROPEAN PATENT SPECIFICATION

(11) **EP 3 050 997 B1**
(45) Date of publication and mention of the grant of the patent: **18.07.2018**
(21) Application number: 13894771.8
(22) Date of filing: 25.09.2013
(51) Int. Cl.: C23C 4/18, C21D 9/08, C21D 9/50, C23C 4/16, C23C 4/10, C23C 4/11

(54) **METHOD FOR DIFFUSION COATING HEAT-RESISTANT METAL MEMBER WITH CREEP REINFORCEMENT MATERIAL, AND CREEP-STRENGTH-ENHANCED HEAT-RESISTANT METAL MEMBER**
VERFAHREN ZUR DIFFUSIONSBESCHICHTUNG EINES HITZEBESTÄNDIGEN METALLELEMENTS MIT KRIECHVERSTÄRKUNGSMATERIAL UND HITZEBESTÄNDIGES METALLELEMENT MIT VERSTÄRKTER KRIECHBESTÄNDIGKEIT
PROCÉDÉ POUR LE REVÊTEMENT PAR DIFFUSION D'UN ÉLÉMENT MÉTALLIQUE RÉSISTANT À LA CHALEUR À L'AIDE DU MATÉRIAU DE RENFORCEMENT DE LA RÉSISTANCE AU FLUAGE ET ÉLÉMENT MÉTALLIQUE RÉSISTANT À LA CHALEUR À RÉSISTANCE AU FLUAGE AMÉLIORÉE

(43) Date of publication of application: 03.08.2016
(73) Proprietor: The Chugoku Electric Power Co., Inc., Hiroshima-shi, Hiroshima 730-8701 (JP)
(72) Inventor: NISHIDA, Hidetaka, Hiroshima-shi Hiroshima 730-8701 (JP)
(74) Representative: Osha Liang
(86) International application number: PCT/JP2013/075927
(87) International publication number: WO 2015/045038

(56) References cited:
- EP-A1- 2 371 986
- JP-A- H 042 761
- JP-A- H1 137 864
- JP-A- H02 277 760
- JP-A- H04 176 856
- JP-A- H08 176 786
- JP-A- 2002 257 163
- JP-A- 2013 136 797
- US-A1- 2009 274 927
- US-A1- 2013 220 523

## Description

### Technical Field

The present invention relates to a method for diffusing and permeating a creep reinforcement material into a heat-resistant metal member, and to a heat-resistant metal member with creep strength enhanced by such a method.

### Background Art

Hitherto, as a method for enhancing creep properties of a heat-resistant metal material, a method has been developed in which, for example, a grain boundary strengthening element that affects creep strength and/or fatigue strength is coated or thermally sprayed to form a film, and heated for a specific duration at a specific temperature (see Japanese Patent No. 3793966).

US2013/0220523 discloses e.g. in example 4 a 430 steel foil was spray coated with a composition comprising e.g. Cr, Mo and B. Then the sprayed foil was put inside a steel pipe i.e. covered by the pipe. The steel foil was pressed against the pipe and the assembly was heat treated in vacuum under 1190-1225 C for 15 to 30 min.

### Summary of Invention

### Technical Problem

An object of the present invention is to provide a method capable of efficiently diffusing and permeating a material that enhances creep strength (hereinafter referred to as a "creep reinforcement material") into a member manufactured using a heat-resistant metal material (hereinafter referred to as a "heat-resistant metal member"), and to provide a heat-resistant metal member with creep strength enhanced by such a method.

### Solution to Problem

In order to address the above problem, according to the present invention, a method for diffusing and permeating a creep reinforcement material into a heat-resistant metal member, and a heat-resistant metal member with creep strength enhanced by such a method, as claimed in claims 1 and 3.

### Advantageous Effects of Invention

The present invention enables provision of a method capable of efficiently diffusing and permeating a creep reinforcement material into a heat-resistant metal member, and provision of a heat-resistant metal member with creep strength enhanced by such a method.

### Brief Description of Drawings

Fig. 1 is a schematic diagram illustrating a method to diffuse and permeate a creep reinforcement material into a heat-resistant metal member, to explain an embodiment of the present invention.
Fig. 2 is a schematic cross-section illustrating a cross-section of Fig. 1, to explain an embodiment of the present invention.

### Description of Embodiments

Detailed explanation follows regarding preferable embodiments of the present invention, with reference to the appended drawings. Note that the objects, features, advantages of the present invention will be clear to a person of ordinary skill in the art from the content of the present specification, and a person of ordinary skill in the art would easily be able to reproduce the present invention from the present specification. The following embodiments, drawings, and the like of the present invention illustrate preferable embodiments of the present invention, and are there to give examples and for the purpose of explanation; however, the present invention is not limited thereto. It will be obvious to a person of ordinary skill in the art that various modifications may be implemented based on the content of the present specification within the scope of the present invention disclosed in the present specification.

Fig. 1 is a schematic diagram illustrating a method for diffusing and permeating a creep reinforcement material into a heat-resistant metal member, to explain an embodiment of the present invention. Fig. 2 is a schematic cross-section illustrating a cross-section of Fig. 1, to explain an embodiment of the present invention. In the present embodiment, explanation is of an example of a case in which an already installed (including repaired cases thereof) or unused, or a degraded, high temperature pipe manufactured using a heat-resistant metal material, is employed as a heat-resistant metal member 10, however, there is no limitation thereto. The heat-resistant metal member 10 may be another high temperature member manufactured using a heat-resistant metal material, such as an already installed (including repaired cases thereof) or unused, or a degraded, turbine.

As illustrated in Fig. 1 and Fig. 2, in the method according to the present invention for diffusing and permeating a creep reinforcement material into a heat-resistant metal member 10, first the creep reinforcement material is coated or thermally sprayed onto a surface of the heat-resistant metal member 10. Then a section 25 onto which the creep reinforcement material has been coated or thermally sprayed is covered by a heat-resistant covering member 30, and the heat-resistant covering member 30 is secured so as to make contact with the section 25. Next, the heat-resistant metal member 10 covered by the heat-resistant covering member 30 is heated for a specific duration at a temperature of 1000°C or greater using a heater 40.

As mentioned above, the heat-resistant metal member 10 coated or thermally sprayed with the creep reinforcement material is covered by the heat-resistant covering member 30 and is heated to a temperature of 1000°C or greater, and thus compressive force acts on the heat-resistant metal member as it thermally expands in a direction toward an outer periphery, restraining thermal expansion of the heat-resistant metal member in the direction toward the outer periphery, and enabling the creep reinforcement material on the surface of the heat-resistant metal member 10 to be efficiently diffused and permeated into the heat-resistant metal member 10. Thus, in cases in which the heat-resistant metal member 10 is a degraded member or an already installed member, by utilizing the force from thermal expansion in the direction toward the outer periphery of the heat-resistant metal member 10, creep voids and cracks in the heat-resistant metal member 10 and a weld 20 thereof are efficiently repaired, enabling regeneration of the heat-resistant metal member 10 and the weld 20 thereof to be achieved. Moreover, structural strengthening of the heat-resistant metal member 10 and the weld 20 thereof can be achieved accompanying restoration of the structure of the heat-resistant metal member 10 and the weld 20 thereof. The creep strength is accordingly enhanced, enabling the lifespan to be extended to that of a new member or greater. On the other hand, in cases in which the heat-resistant metal member 10 is an unused member, structural strengthening of the heat-resistant metal member 10 and the weld 20 thereof can be achieved, thereby enhancing the creep strength and enabling the lifespan to be extended to that of a new member or greater.

In the method for diffusing and permeating a creep reinforcement material into the heat-resistant metal member 10 according to the present invention, etching treatment, or shot peening and etching treatment, may be performed on the section 25 to be coated or thermally sprayed with the creep reinforcement material prior to coating or thermally spraying the creep reinforcement material on the surface of the heat-resistant metal member 10. Such processing enables work hardening of the surface layer of the heat-resistant metal member 10 to be performed by plastic deformation, enables residual compressive stress to be imparted to the surface of the heat-resistant metal member 10, and enables any oxidized film on the surface of the heat-resistant metal member 10 to be removed.

In the method for diffusing and permeating a creep reinforcement material into the heat-resistant metal member 10 according to the present invention, processing to remove (reduce) residual stress, such as stress relief or tension annealing processing, may be performed after the heat-resistant metal member 10 covered by the heat-resistant covering member 30 has been heated to a temperature of 1000°C or greater using the heater 40. More specifically, after the heat-resistant metal member 10 covered by the heat-resistant covering member 30 has been heated to a temperature of 1000°C or greater using the heater 40, the heat-resistant metal member 10 may be first cooled to room temperature, then reheated to a temperature of an A₁ transformation point or greater (preferably from 10°C to 100°C above 1000°C) for a specific duration (for example, from approximately several hours to approximately 24 hours).

Moreover, in the method to diffuse and permeate a creep reinforcement material into the heat-resistant metal member 10 according to the present invention, in order to restrict thermal expansion of the heat-resistant metal member 10 toward the outside in the length direction thereof (in directions toward the ends of the heat-resistant metal member 10) occurring when the heat-resistant metal member 10, which has been coated or thermally sprayed with the creep reinforcement material, is covered by the heat-resistant covering member 30 and heated by the heater 40, the heat-resistant metal member 10 may be secured in sections not being heated by the heater 40, by, for example, two clamps so as to sandwich the section being heated by the heater 40.

In cases in which the section heated by the heater 40 is small compared to the overall heat-resistant metal member 10, there is no need to secure the heat-resistant metal member 10 in sections not being heated by the heater 40 with clamps or the like, since thermal expansion toward the outside in the length direction of the heat-resistant metal member 10 in the section being heated by the heater 40 is restricted by the sections not being heated by the heater 40.

According to the invention the heat-resistant metal of the member 10 is made of 0.3Mo steel, 0.5Mo steel, 0.5Cr-0.5Mo steel, 1Cr-0.2Mo steel, 1Cr-0.5Mo steel, 1.25Cr-0.5Mo steel, 2.25Cr-1Mo steel, 5Cr-0.5Mo steel, 7Cr-0.5Mo steel, 9Cr-1Mo steel, 0.3Cr-Mo-V steel, 0.5Cr-Mo-V steel, 9Cr-Mo-V steel, 12Cr-Mo-V steel, 1Cr-1.25Mo-0.25V steel, 9Cr-1Mo-W steel, SUS304, SUS304L, SUS316, SUS316L, SUS316TI, SUS317, SUS321, SUS347H, SUS310S, Super304, SUS904L, NCF600, NCF601, NCF800, and NCF800H.

The creep reinforcement material needs to contain an element which has a melting point of 1000°C or greater and in which precipitation strengthening and solid solution strengthening occur upon heating to a temperature of 1000°C or greater so as to enable creep strength to be enhanced. According to the invention, the heat-resistant metal member 10, the creep reinforcement material contains one or a plurality of elements appropriately selected from B (boron), W (tungsten), Cr (Chromium), Mo (molybdenum), Nb (niobium), V (vanadium), Hf (hafnium), Zr (zirconium), Ti (titanium), Cu (copper), and Co (cobalt). In cases in which the creep reinforcement material is coated on the surface of the heat-resistant metal member 10, powdered creep reinforcement material may be employed as it is, or a coating agent of the creep reinforcement material in a liquid form or paste form using a binder, solvent, adhesive or the like may be employed. In cases in which the creep reinforcement material is thermally sprayed on the surface of the heat-resistant metal member 10, for example, a known thermal spray method may be appropriately employed, such as a plasma spraying method using powdered creep reinforcement material. Note that coating or thermally spraying of the creep reinforcement material on the surface of the heat-resistant metal member 10 may be performed over the entire outer peripheral surface of the heat-resistant metal member 10 as in the present embodiment, or may be performed on a part of the surface of the heat-resistant metal member 10.

The heat-resistant covering member 30 needs to be capable of covering the section 25 coated or thermally sprayed with the creep reinforcement material so as to make contact with the section 25, as long as it is made from a heat-resistant material that restrains thermal expansion in the section 25 in the direction toward the outer periphery of the heat-resistant metal member 10 occurring when heated to the heating temperature mentioned above, and is able to maintain the approximate profile of the heat-resistant metal member 10 at the section 25. A material having a lower thermal expansion coefficient than the heat-resistant metal member 10 at temperatures of the heating temperature mentioned above or greater is preferably employed for the heat-resistant covering member 30. In cases in which the heat-resistant covering member 30 is configured from a heat-resistant material different from that of the heat-resistant metal member 10, yet having a thermal expansion coefficient of about the same as the heat-resistant metal member 10, or from a heat resistant material having a higher thermal expansion coefficient than the heat-resistant metal member 10, in order to restrain the thermal expansion of the heat-resistant covering member 30 occurring when heated to the heating temperature mentioned above, the outer periphery of the heat-resistant covering member 30 may be secured by a member of a heat-resistant material having a lower thermal expansion coefficient than the heat-resistant metal member 10 at or above the heating temperature mentioned above, so as to maintain the profile of the heat-resistant covering member 30.

According to the invention, the heat-resistant covering member 30 being a ceramic or an alloy, including ceramics such as alumina, zirconia, aluminum nitride, silicon carbide, silicon nitride, cordierite, sialon, zircon, and mullite, and alloys such as Alloy 903, Alloy 909, and HRA 929.

The heat-resistant covering member 30 is, for example, of a cord, plate, or clamp shape. Securing of the above may be performed by, for example, wrapping a cord-shaped or plate-shaped heat-resistant covering member 30 around the outer periphery of the heat-resistant metal member 10 at the section 25 coated or thermally sprayed with the creep reinforcement material, by attaching a clamp-shaped heat-resistant covering member 30 to the outer periphery of the heat-resistant metal member 10 at the section 25 coated or thermally sprayed with the creep reinforcement material, or by attaching a heat-resistant covering member 30 formed in a plate shape or the like to the outer periphery of a heat-resistant metal member 10 at the section 25 coated or thermally sprayed with the creep reinforcement material using fasteners, such as clamps or screws. In the present embodiment, the heat-resistant covering member 30 is made from fittings including two substantially semi-circular arc cross-section shapes. The heat-resistant covering member 30 is then secured to the surface of the heat-resistant metal member 10 using threaded members 35 attached to flanges of these fittings, such that the inner face of the fittings contact the outer periphery of the heat-resistant metal member 10 at the section 25 coated or thermally sprayed with the creep reinforcement material. The threaded members 35 are manufactured, for example, from the same material as the heat-resistant covering member 30.

The heating temperature of the heat-resistant metal member 10 coated or thermally sprayed with the creep reinforcement material is a temperature of 1000°C or greater. Preferably the heat-resistant metal member 10 is heated at a temperature of, or greater than, an A₃ transformation point of the component of the heat-resistant metal material of the member 10 or the creep reinforcement material having the highest A₃ transformation point (preferably from 10°C to 100°C above 1000°C) for a specific duration (for example, from approximately several hours to approximately 24 hours) . Note that although the present embodiment employs, as a heating device, the high frequency heater 40, which is capable of heating the heat-resistant metal member 10 coated or thermally sprayed with the creep reinforcement material, from the outer periphery thereof, there is no particular limitation thereto, as long as a heating device capable of heating the heat-resistant metal member 10 at the section 25 coated or thermally sprayed with the creep reinforcement material.

The product of diffusing and permeating the creep reinforcement material into the heat-resistant metal member 10 by the method described above is useful as a heat-resistant metal member with enhanced creep strength due to the creep strength being enhanced as described above.

### Reference Signs List

10 heat-resistant metal member
20 weld
25 section coated or thermally sprayed with creep reinforcement material
30 heat-resistant covering member
35 threaded member
40 high frequency heater

## Claims

1. A method for diffusing and permeating a creep reinforcement material into a heat-resistant metal member, the method comprising:
coating or thermally spraying a creep reinforcement material onto a surface of a heat-resistant metal member;
covering, by a heat-resistant covering member, a section coated or thermally sprayed with the creep reinforcement material, and securing the heat-resistant covering member so as to contact the section; and
heating the heat-resistant metal member covered by the heat-resistant covering member to a temperature of 1000°C or greater,
the creep reinforcement material containing one or a plurality of elements selected from B, W, Cr, Mo, Nb ,V, Hf, Zr, Ti, Cu, and Co,
the heat-resistant metal member being made of 0.3Mo steel, 0.5Mo steel, 0.5Cr-0.5Mo steel, 1Cr-0.2Mo steel, 1Cr-0.5Mo steel, 1.25Cr-0.5Mo steel, 2.25Cr-1Mo steel, 5Cr-0.5Mo steel, 7Cr-0.5Mo steel, 9Cr-1Mo steel, 0.3Cr-Mo-V steel, 0.5Cr-Mo-V steel, 9Cr-Mo-V steel, 12Cr-Mo-V steel, 1Cr-1.25Mo-0.25V steel, 9Cr-1Mo-W steel, SUS304, SUS304L, SUS316, SUS316L, SUS316TI, SUS317, SUS321, SUS347H, SUS310S, Super304, SUS904L, NCF600, NCF601, NCF800, or NCF800H,
the heat-resistant covering member being a ceramic or an alloy.

2. The method according to claim 1, wherein,
after heating the heat-resistant metal member covered by the heat-resistant covering member to a temperature of 1000°C or greater, the heat-resistant metal member covered by the heat-resistant covering member is cooled and re-heated to a temperature of an A₁ transformation point or greater.

3. A heat-resistant metal member with enhanced creep strength,
the heat-resistant metal member (10) being obtained by
coating or thermally spraying a creep reinforcement material (25) onto a surface of a heat-resistant metal member,
covering, by a heat-resistant covering member (30), a section coated or thermally sprayed with the creep reinforcement material, and securing the heat-resistant covering member so as to contact the section, and
heating the heat-resistant metal member covered by the heat-resistant covering member to a temperature of 1000°C or greater; and
the creep reinforcement material (25) containing one or a plurality of elements selected from B, W, Cr, Mo, Nb, V, Hf, Zr, Ti, Cu, and Co,
the heat-resistant metal member (10) being made of 0.3Mo steel, 0.5Mo steel, 0.5Cr-0.5Mo steel, 1Cr-0.2Mo steel, 1Cr-0.5Mo steel, 1.25Cr-0.5Mo steel, 2.25Cr-1Mo steel, 5Cr-0.5Mo steel, 7Cr-0.5Mo steel, 9Cr-1Mo steel, 0.3Cr-Mo-V steel, 0.5Cr-Mo-V steel, 9Cr-Mo-V steel, 12Cr-Mo-V steel, 1Cr-1.25Mo-0.25V steel, 9Cr-1Mo-W steel, SUS304, SUS304L, SUS316, SUS316L, SUS316TI, SUS317, SUS321, SUS347H, SUS310S, Super304, SUS904L, NCF600, NCF601, NCF800, or NCF800H,
the heat-resistant covering member (30) being a ceramic or an alloy.

4. The heat-resistant metal member according to claim 3, wherein
the heat-resistant metal member is obtained by, after heating the heat-resistant metal member covered by the heat-resistant covering member to a temperature of 1000°C or greater, cooling and re-heating to a temperature of an A₁ transformation point or greater.

## Patentansprüche

1. Verfahren zum Diffusionsbeschichten und Permeieren eines hitzebeständigen Metallelements mit einem Kriechverstärkungsmaterial, wobei das Verfahren umfasst:
Beschichten oder thermisches Spritzen eines Kriechverstärkungsmaterials auf eine Oberfläche eines hitzebeständigen Metallelements;
Bedecken, durch ein hitzebeständiges Deckelement, eines Abschnitts, der mit dem Kriechverstärkungsmaterial beschichtet oder thermisch gespritzt ist, und Sichern des hitzebeständigen Abdeckelements, so dass es den Abschnitt berührt; und
Erhitzen des hitzebeständigen Metallelements, das durch das hitzebeständige Abdeckelement bedeckt ist, auf eine Temperatur von 1000 °C oder mehr,
wobei das Kriechverstärkungsmaterial eines oder eine Vielzahl von Elementen ausgewählt aus B, W, Cr, Mo, Nb, V, Hf, Zr, Ti, Cu, und Co enthält,
wobei das hitzebeständige Metallelement aus 0,3Mo Stahl, 0,5Mo Stahl, 0,5Cr-0,5Mo Stahl, 1Cr-0,2Mo Stahl, 1Cr-0,5Mo Stahl, 1,25Cr-0,5Mo Stahl, 2,25Cr-1Mo Stahl, 5Cr-0,5Mo Stahl, 7Cr-0,5Mo Stahl, 9Cr-1Mo Stahl, 0,3Cr-Mo-V Stahl, 0,5Cr-Mo-V Stahl, 9Cr-Mo-V Stahl, 12Cr-Mo-V Stahl, 1Cr-1,25Mo-0,25V Stahl, 9Cr-1Mo-W Stahl, SUS304, SUS304L, SUS316, SUS316L, SUS316TI, SUS317, SUS321, SUS347H, SUS310S, Super304, SUS904L, NCF600, NCF601, NFC800, oder NCF800H gefertigt ist,
wobei das hitzebeständige Abdeckelement eine Keramik oder eine Legierung ist.

2. Verfahren nach Anspruch 1, wobei
nach dem Erhitzen des hitzebeständigen Metallelements, das durch das hitzebeständige Abdeckelement bedeckt ist, auf eine Temperatur von 1000 °C oder mehr das durch das hitzebeständige Abdeckelement bedeckte hitzebeständige Metallelement abgekühlt wird und wieder auf eine Temperatur eines A₁ Transformationspunkts oder höher erhitzt wird.

3. Hitzebeständiges Metallelement mit verbesserter Kriechfestigkeit, wobei das hitzebeständige Metallelement (10) erhalten wird durch
Beschichten oder thermisches Spritzen eines Kriechverstärkungsmaterials (25) auf eine Oberfläche eines hitzebeständigen Metallelements,
Bedecken eines Abschnitts, der mit dem Kriechverstärkungsmaterial beschichtet oder thermisch bespritzt ist, durch ein hitzebeständiges Abdeckelement (30), und Sichern des hitzebeständigen Abdeckelements, so dass es den Abschnitt berührt, und
Erhitzen des hitzebeständigen Metallelements, das durch das hitzebeständige Abdeckelement bedeckt wird, auf eine Temperatur von 1000 °C oder mehr; und
wobei das Kriechverstärkungsmaterial (25) eines oder eine Vielzahl von Elementen ausgewählt aus B, W, Cr, Mo, Nb, V, Hf, Zr, Ti, Cu, und Co enthält,
wobei das hitzebeständige Metallelement (10) aus 0,3Mo Stahl, 0,5Mo Stahl, 0,5Cr-0,5Mo Stahl, 1Cr-0,2Mo Stahl, 1Cr-0,5Mo Stahl, 1,25Cr-0,5Mo Stahl, 2,25Cr-1Mo Stahl, 5Cr-0,5Mo Stahl, 7Cr-0,5Mo Stahl, 9Cr-1Mo Stahl, 0,3Cr-Mo-V Stahl, 0,5Cr-Mo-V Stahl, 9Cr-Mo-V Stahl, 12Cr-Mo-V Stahl, 1Cr-1,25Mo-0,25V Stahl, 9Cr-1Mo-W Stahl, SUS304, SUS304L, SUS316, SUS316L, SUS316TI, SUS317, SUS321, SUS347H, SUS310S, Super304, SUS904L, NCF600, NCF601, NFC800, oder NCF800H gefertigt ist,
wobei das hitzebeständige Abdeckelement (30) eine Keramik oder eine Legierung ist.

4. Hitzebeständiges Metallelement nach Anspruch 3, wobei
das hitzebeständige Metallelement erhalten wird durch, nach dem Erhitzen des durch das hitzebeständige Abdeckelement bedeckten hitzebeständigen Metallelements auf eine Temperatur von 1000 °C oder mehr, Abkühlen und Wiedererhitzen auf eine Temperatur eines A₁-Transformationspunktes oder mehr.

## Revendications

1. Procédé de diffusion et de perméation d'un matériau de renforcement de la résistance au fluage dans un élément métallique résistant à la chaleur, ledit procédé comprenant :
le revêtement ou la pulvérisation thermique d'un matériau de renforcement de la résistance au fluage sur une surface d'un élément métallique résistant à la chaleur ;
l'application d'un élément de couverture résistant à la chaleur sur une section revêtue ou ayant reçu une pulvérisation thermique de matériau de renforcement de la résistance au fluage, et la fixation de l'élément de couverture résistant à la chaleur de sorte qu'il soit en contact avec la section ; et
le chauffage de l'élément métallique résistant à la chaleur recouvert de l'élément de couverture résistant à la chaleur à une température de 1000 °C ou plus,
le matériau de renforcement de la résistance au fluage contenant un ou une pluralité des éléments choisis parmi B, W, Cr, Mo, Nb, V, Hf, Zr, Ti, Cu et Co,
l'élément métallique résistant à la chaleur étant constitué d'acier 0,3 Mo, d'acier 0,5 Mo, d'acier 0,5 Cr-0,5 Mo, d'acier 1 Cr-0,2 Mo, d'acier 1 Cr-0,5 Mo, d'acier 1,25 Cr-0,5 Mo, d'acier 2,25 Cr-1 Mo, d'acier 5 Cr-0,5 Mo, d'acier 7 Cr-0,5 Mo, d'acier 9 Cr-1 Mo, d'acier 0,3 Cr-Mo-V, d'acier 0,5 Cr-Mo-V, d'acier 9 Cr-Mo-V, d'acier 12 Cr-Mo-V, d'acier 1 Cr-1,25 Mo-0,25 V, d'acier 9 Cr-1 Mo-W, SUS 304, SUS 304L, SUS 316, SUS 316L, SUS 316TI, SUS 317, SUS 321, SUS 347H, SUS 310S, Super 304, SUS 904L, NCF 600, NCF 601, NCF 800 ou NCF 800H,
l'élément de couverture résistant à la chaleur étant une céramique ou un alliage.

2. Procédé selon la revendication 1, dans lequel après le chauffage de l'élément métallique résistant à la chaleur recouvert de l'élément de couverture résistant à la chaleur à une température de 1000 °C ou plus, l'élément métallique résistant à la chaleur recouvert de l'élément de couverture résistant à la chaleur est refroidi, puis chauffé à nouveau jusqu'à une température d'un point de transformation A₁ ou plus.

3. Elément métallique résistant à la chaleur à résistance au fluage améliorée,
ledit élément métallique résistant à la chaleur (10) étant obtenu par
revêtement ou pulvérisation thermique d'un matériau de renforcement de la résistance au fluage (25) sur une surface d'un élément métallique résistant à la chaleur ;
application d'un élément de couverture résistant à la chaleur (30), sur une section revêtue ou ayant reçu une pulvérisation thermique du matériau de renforcement de la résistance au fluage, et fixation de l'élément de couverture résistant à la chaleur de sorte qu'il soit en contact avec la section ; et
chauffage de l'élément métallique résistant à la chaleur recouvert de l'élément de couverture résistant à la chaleur à une température de 1000 °C ou plus, et le matériau de renforcement de la résistance au fluage (25) contenant un ou une pluralité des éléments choisis parmi B, W, Cr, Mo, Nb, V, Hf, Zr, Ti, Cu et Co,
l'élément métallique résistant à la chaleur étant constitué d'acier 0,3 Mo, d'acier 0,5 Mo, d'acier 0,5 Cr-0,5 Mo, d'acier 1 Cr-0,2 Mo, d'acier 1 Cr-0,5 Mo, d'acier 1,25 Cr-0,5 Mo, d'acier 2,25 Cr-1 Mo, d'acier 5 Cr-0,5 Mo, d'acier 7 Cr-0,5 Mo, d'acier 9 Cr-1 Mo, d'acier 0,3 Cr-Mo-V, d'acier 0,5 Cr-Mo-V, d'acier 9 Cr-Mo-V, d'acier 12 Cr-Mo-V, d'acier 1 Cr-1,25 Mo-0,25 V, d'acier 9 Cr-1 Mo-W, SUS 304, SUS 304L, SUS 316, SUS 316L, SUS 316TI, SUS 317, SUS 321, SUS 347H, SUS 310S, Super 304, SUS 904L, NCF 600, NCF 601, NCF 800 ou NCF 800H,
l'élément de couverture résistant à la chaleur (30) étant une céramique ou un alliage.

4. Elément métallique résistant à la chaleur selon la revendication 3, dans lequel
l'élément métallique résistant à la chaleur est obtenu, après le chauffage de l'élément métallique résistant à la chaleur recouvert de l'élément de couverture résistant à la chaleur à une température de 1000 °C ou plus, en le refroidissant, puis en le chauffant à nouveau jusqu'à une température d'un point de transformation A₁ ou plus.
